

## UNITED STATES PATENT OFFICE

EMIL C. LOETSCHER, OF DUBUQUE, IOWA

## METHOD OF TREATING VENEER

No Drawing.

Application filed August 22, 1931. Serial No. 558,836.

The object of this invention is to overcome the great difficulty encountered with thin natural wood veneer when used with phenol condensation products, caused by natural resins in the veneer uniting with the phenol condensation products producing a sticky substance which causes the product to adhere so firmly to the press platen that it cannot, in many cases be removed therefrom, without 10 tearing the wood veneer and the product to pieces.

While this does not happen with all woods, it is particularly common in the cases of walnut and of oak. It depends somewhat upon 15 the nature of the wood and the amount of resin in the wood.

It is obvious that in veneering panels or other articles by a process which employs phenol condensation products as a cementing 20 material as well as a finish, that even a slight spot-sticking of the veneer would spoil the product, since no way has been discovered by which the spot can be finished to the same high degree and polish of the finish of the 25 material surrounding the spot. In many cases the adhesion is so strong that the veneer, together with part of the base or core material is torn to pieces. Even if only a small percentage of the work causes trouble 30 from this source, it would make an impractical operation in using phenol condensation products because the work which is spotted is a total loss.

The present invention, in addition to preventing sticking of veneer to the press platen, 35 has the further advantage of materially removing the color of the veneer and of replacing the same by stains which give the exact and uniform shade of color desired. Some 40 natural woods change in color, due to the heat of the process of applying phenol condensation products, and by removing the color with a bleaching agent, the correct color can be restored with a suitable stain or stains 45 or aniline dyes.

In practicing the method of this invention in connection with thin wood veneers, (in most cases 1/100" in thickness,) the veneer sheets are arranged vertically in racks and 50 immersed in an agitated or circulated solu-

tion capable of removing the natural resins from and of bleaching the veneer. A 5% solution of sodium hydroxide is satisfactory for the purposes though harsh on the veneer, and a more satisfactory solution consists of 55 2½% solution of sodium carbonate with 2½% sodium bicarbonate. Sodium perborate also fills the requirements. Other agents, such as ordinary bleaching powder, calcium hydroxide, ammonium carbonate, and potassium permanganate have each been found effective, and applicant does not care to be restricted to any particular chemical, but desires to cover any agent for producing the 60 stated result.

After the veneer sheets have been soaked or treated in any of these solutions, they are removed to another tank and thoroughly washed with water to remove all traces of the 65 chemicals. The veneers are then allowed to 70 drain.

The treated veneers may now be applied in their bleached state to the base or core material, but if they are to be colored, they are immersed, preferably edgeways in vertical 75 position, into a vat containing a solution of ordinary wood stains, preferably of the permanent stain type, or suitable aniline dyes. After dyeing, the veneers are removed from the color solution and dried, preferably between sheets of absorbent basswood heated to a temperature of 150° F. or 200° F. and arranged flatways to avoid wrinkling or 80 curling.

The veneer sheets are now coated, by immersion or otherwise, on both sides with phenol formaldehyde condensation product, such as bakelite, after which they are heated at a moderate temperature of about 130° C. 85 for six to ten minutes to remove most of the solvent therefrom. The veneers are then 90 ready to be applied to the base or core material and subjected to pressure, between platens of a hydraulic press, in the presence of 95 heat sufficient to react the condensation product. The condensation product on one side of the veneer cements it to the base or core material, while the condensation product on 100 the side of the veneer next to the press platen

produces a varnish like finish coating on the exposed side of its veneer.

The heat and pressure employed to react the phenol condensation product would soften 5 and cause natural resins to be forced from the cells of the wood veneer and by materially removing these natural resins, as above outlined, they are not present to break through or to unite with the finish coating to 10 form the sticky substance that causes the veneer to stick to the press platen and cause surface spots that spoil the product.

Further, there will be no discolorations of 15 the veneer, due to the temperature of the press platens causing some of the natural resins to react with the condensation product to cause dark discolorations, which are quite objectionable.

When the veneers are treated in this manner, the color thereof is very uniform and 20 very much more beautiful than when the natural untreated veneers are used, even though the latter could be removed from the press platens without sticking.

25 Apart from its more important utility in connection with wood veneers, the invention has considerable value in connection with any cellulosic product having a surface coating of phenol condensation product wherein there 30 is danger of the natural resins of the cellulosic material uniting with the phenol condensation product to cause spot sticking as in the case of veneered products.

35 While the term platen has been adopted herein, it is not intended that its meaning should be restricted to a flat plate-like body, but that it should be accepted in its broader sense as meaning any surface whether plain or ornamental with which the product is 40 pressed while the condensation product is being reacted to give it shape and from which the finished product must be readily released.

What I claim is:—

45 1. The method of coating an article containing cellulosic material with condensation product, consisting in removing natural resin from the cellulosic material then treating the cellulosic material with condensation 50 product in a manner to produce a film of the latter on the surface of the finished article, and subjecting the treated cellulosic material to platen pressure and heat to react the condensation product.

55 2. The method of forming an article having a condensation-product-coated covering of cellulosic material, consisting in removing natural resin from the cellulosic material, then treating the cellulosic material with condensation 60 product in a manner to produce a film of the latter on the exposed surface of the finished article, applying the treated cellulosic material to a base with condensation product interposed, and subjecting the cel-

in the presence of heat sufficient to react the condensation product.

3. The method of forming an article having a condensation-product-coated wood veneering, consisting in removing natural resin 70 from wood veneer, then treating the wood veneer with condensation product in a manner to produce a film of the latter on the exposed surface of the finished article, applying the treated wood veneer to a base 75 with an adhesive and subjecting the veneer and base to platen pressure in the presence of heat sufficient to react the condensation product.

4. The method of coating wood with condensation product, consisting in treating the wood with a bleaching agent having the property of removing natural resin from the wood, then treating the wood with condensation product in a manner to produce a film 80 of the latter on the surface of the finished product, and then subjecting the wood to platen pressure in the presence of heat sufficient 85 to react the condensation product.

5. The method of coating wood with condensation product, consisting in treating the wood with a bleaching agent having the property of removing natural resin from the wood, coloring the wood, then treating the wood with condensation product in a manner to 90 produce a film of the latter on the surface of the finished product, and then subjecting the wood to platen pressure in the presence of heat sufficient to react the condensation product.

In testimony whereof I affix my signature.  
EMIL C. LOETSCHER.

105

110

115

120

125

130